

Sept. 21, 1926.

1,600,257

C. K. TOPPING

MANUFACTURE OF COPPER STRIPS OR BARS

Filed May 29, 1925



INVENTOR  
Charles K. Topping  
BY  
Pennie, Davis, Martin & Edwards  
ATTORNEYS

Patented Sept. 21, 1926.

1,600,257

# UNITED STATES PATENT OFFICE.

CHARLES K. TOPPING, OF NEWBURGH, NEW YORK, ASSIGNOR TO CHILE EXPLORATION COMPANY, OF NEW YORK, N. Y., A CORPORATION OF NEW JERSEY.

## MANUFACTURE OF COPPER STRIPS OR BARS.

Application filed May 29, 1925. Serial No. 33,661.

This invention relates to the manufacture of metallic plates, sheets, strips, bars or the like, and more particularly to the manufacture of copper articles of the character mentioned. The invention has for its object the provision of an improved method of making metallic, and more particularly copper, plates, sheets, strips, bars and the like, as well as the provision as a new article of manufacture of metallic articles resulting from the practice of the improved method of the invention.

In accordance with the invention, metallic (and more particularly copper) plates, sheets, strips, bars, or the like, are produced by the electrodeposition of the metal, such as copper, upon an appropriate metallic starting blank. The metallic starting blank is also preferably made of electrodeposited metal. The invention thus contemplates the electrodeposition of a thin layer of metal, such as copper, upon an appropriate form. The thin layer of electrodeposited metal is then stripped from the form and progressively passed through an electrodepositing apparatus. While passing through the electrodepositing apparatus, the starting blank or initial layer of electrodeposited metal is built up to the desired thickness by electrodeposition, and the resulting plate of electrodeposited metal is progressively withdrawn from the electrodepositing apparatus.

The improved method of the invention thus comprises two steps, in the first of which a starting blank is produced, preferably by electrodeposition, and in the second step of which the starting blank is built up of electrodeposited metal to a desired thickness. In the preferred practice of the invention, the starting blank is continuously produced by electrodeposition upon a rotating form and is continuously stripped from the form and wound on a spool, or otherwise, appropriately disposed of. In this manner, an electrodeposited starting blank of any appropriate width and of any desired length may be advantageously produced. The starting blank is then progressively passed through an electrodepositing apparatus during which passage electrodeposition of metal takes place until a sufficient thickness of electrodeposited metal has been obtained. The progress of the starting blank through the electrodepositing apparatus is so regu-

lated that this desired thickness of electrodeposited metal is obtained during the time any portion of the starting blank is passing between the entrance and exit ends of the electrodepositing apparatus.

The invention is particularly applicable 60 for making bus-bar copper, that is, the bars or laminæ for building up copper bus-bars for conducting electric current of relatively high amperage. Heretofore, it has been customary to make the copper bars or laminæ for bus bars by rolling. The rolling operation is relatively expensive and necessitates the provision of a copper rolling mill. Bus bars or laminæ of electrodeposited copper can be economically and advantageously 70 manufactured in accordance with the present invention. Moreover, the electrical conductivity of the electrodeposited metal is, in most cases, higher than that of the rolled metal. 75

The novel features of the invention and my present preferred mode of practicing the invention will be best understood from the following description taken in conjunction with the accompanying drawings. I will hereinafter particularly describe the invention as applied to the manufacture of copper plates, sheets, strips, bars, or the like, but it is to be understood that the principles of the invention are applicable to the production of articles of this general character made of metals other than copper. 85

In the accompanying drawings, Fig. 1 is a sectional end elevation, and Fig. 2 is a sectional front elevation of an apparatus 90 for forming a starting blank, and Fig. 3 is a sectional elevation of an electrodepositing apparatus for carrying out the aforementioned second step of the invention.

Referring first to Figs. 1 and 2 of the 95 drawings, there is diagrammatically illustrated an electrolytic tank 5 of wood, concrete or other appropriate material. The tank has a substantially semi-cylindrical lining 6 of lead, or other appropriate material resistant to the action of the acid electrolyte. Where the lining 6 is of lead, it may serve as the anode and is electrically connected to the positive terminal of an appropriate source of direct current energy. 100 The tank is provided with an inlet pipe 7 for introducing fresh electrolyte and an overflow or outlet pipe 8 for withdrawing 105

electrolyte from the tank. A perforated pipe 9 is provided near or on the bottom of the tank through which air or other appropriate gas may be introduced into the electrolyte for the purpose of agitation.

A cylindrical form is rotatably mounted within the tank 5. This form is built up of a plurality of metallic rings 10 spaced apart by relatively thin disks 11 of insulating material. The rings 10 and disks 11 are clamped or otherwise appropriately secured together on a metallic shaft 12 journaled in the ends of the tank 5. The end rings 10 are covered with disks of insulating material 11'. The rings 10 may conveniently be made of copper and have a smooth or polished cylindrical surface. This cylindrical surface is preliminarily treated with some appropriate "dope," such as rack grease, sal ammoniac and mercury, for preparing the surface for the electrodeposition of copper thereon and the stripping of the electrodeposited copper therefrom.

A pulley 13 is secured to the shaft 12 and is connected to any appropriate source of power for slowly rotating the cylindrical form (10-11). In practice, this form makes approximately one complete revolution in 24 hours, although it is to be understood that the form may be rotated at a different rate, depending upon the particular conditions of electrodeposition existing or desired.

A slip ring 14 is secured to the shaft 12. A stationary brush 15 contacts with the slip ring 14 and is electrically connected to the negative terminal of the source of direct current energy employed for the electrodepositing operation. Thus, the rings 10 are electrically connected together and to the brush 15 and constitute the cathode of the electrolytic apparatus.

The lower half of the cylindrical form 10-11 is submerged in an appropriate copper electrolyte in the tank 5. This electrolyte may conveniently be of the following composition:

35 grams of copper per liter  
100 grams sulfuric acid per liter  
50 0.03 grams of chlorine per liter.

Mounted above the tank 5 are a plurality of rotatable spools 16 upon which are wound the electrodeposited starting blanks stripped from the form 10-11. In the operation of the apparatus illustrated in Figs. 1 and 2 of the drawings, the copper electrolyte is passed through the tank 5 and is appropriately agitated while in the tank in order to provide an electrolyte of substantially uniform composition. Copper is continuously electrodeposited upon that portion of the rotating cylindrical form which is submerged in the electrolyte. In the apparatus illustrated in Figs. 1 and 2, five separate strips of copper are simultaneously electro-

deposited. As the rotation of the cylindrical form, in the direction of the arrows in Figs. 1 and 2, carries the thin layer of electrodeposited copper out of the electrolyte, the electrodeposited copper is stripped from the form and wound on the spools 16. This stripping of the electrodeposited copper from the form and winding on the spools may be done manually and from time to time as necessary. In this manner, there is continuously formed strips, sheets, or the like, of appropriate thickness, say one-thirtieth of an inch, and of any desired length, which serve as starting blanks in the second step of the improved method of the invention.

The electro-depositing apparatus of Fig. 3 comprises a long tank 17 of wood, concrete or other appropriate material. This tank is lined with lead, mastic, or the like, to resist the corrosive action of the acid electrolyte. The electrolyte is continuously supplied near the bottom of the tank and through an inlet pipe 18 and continuously overflows through an outlet pipe 19. One or more perforated agitating pipes 20, adapted to be supplied with compressed air, are provided near the bottom of the tank 17.

The spools of starting blanks 21 (initially formed and wound up on the spools 16 as hereinbefore described) are appropriately mounted for progressive and continuous passage through the copper electrolyte in the tank 17. To this end, the starting blanks pass over guide rolls 22 and enter one end of the tank 17. A liquid seal 23 is provided in the end of the tank 17 for each starting blank, so that the blanks may freely pass through the end of the tank while the escape of electrolyte from the tank is substantially inhibited.

Within the tank 17 the starting blanks are arranged in superposed horizontal planes. Each starting blank passes between two horizontally disposed lead anode plates 24. The lead anode plates are electrically connected together and to the positive terminal of an appropriate source of direct current energy, as diagrammatically indicated by reference character 25 in Fig. 3. The copper starting blanks are similarly electrically connected together and to the negative terminal of the source of direct current energy employed for the electrodepositing operation, as diagrammatically indicated by reference character 26 in Fig. 3.

The finished plates of electrodeposited copper are progressively and continuously withdrawn through the exit end of the tank 17. To this end, the superposed plates of electrodeposited copper pass through liquid seals 27 in the end of the tank 17 and are clamped to a yoke 28. The yoke 28 is connected in any appropriate manner, as, for example, by a block and tackle 29, to an appropriate source of power (not shown) for

progressively pulling the starting blanks on said blank an electrodeposit of metal of with their accumulating deposit of copper a desired thickness.

5 The starting blanks enter the electrodepositing tank and in the course of their passage through the electrolyte in the tank receive on each side thereof an appropriate deposit of copper. The rate of travel of the copper blanks through the tank is regulated so that a deposit of the desired thickness is obtained by the time the blank reaches the exit end of the tank. The copper electrolyte is preferably of the same composition as hereinbefore described.

5 When the spools of starting blanks 21 have been completely unwound, a fresh spool may be joined thereto by riveting, crimping, welding, brazing, or in any other appropriate manner. Similarly, when a desired 10 length of finished copper plate or sheet has been discharged through the exit end of the tank, the plates or sheets may be cut and the yoke again fastened to the plates or sheets projecting through the exit end of the tank. 15 In this manner the operation of building up the copper plates or sheets is substantially continuous, and plates or sheets of any desired length may be produced.

In making bus-bar copper, the rings 10, 20 of the forming cylinder, may conveniently be ten inches in width and fifty inches in diameter. Approximately 100 feet of starting blank may be wound on the spools 16. The tank 17 may conveniently be about 100 25 feet long, 16 inches high and 20 inches wide. The plates or sheets withdrawn from the tank 17 may be one-fourth inch, or more, as desired, in thickness. Preferably, these withdrawn plates or sheets are cut in lengths 30 of about 100 feet. These particular dimensions are given merely as illustrative of the invention and are in no sense to be regarded as restrictive.

15 In the appended claims I have used the term "plate" to designate a plate-like article, and intend to include therein sheets, strips, bars and the like.

I claim:—

1. The method of manufacturing metallic plates or the like which comprises forming a metallic starting blank, and progressively passing said starting blank through an electrodepositing apparatus in the course of which there is built up on said blank an electrodeposit of metal of a desired thickness.

2. The method of manufacturing metallic plates or the like which comprises electrodepositing a thin layer of metal upon an appropriate form, stripping the layer of electrodeposited metal from said form and thereby producing a metallic starting blank, and progressively passing said starting blank through an electrodepositing apparatus in the course of which there is built up

70 3. The method of manufacturing copper plates or the like which comprises forming a metallic starting blank, and progressively passing said starting blank through a copper electrodepositing apparatus in the course of which there is built up on said blank an electrodeposit of copper of a desired thickness.

75 4. The method of manufacturing copper plates or the like which comprises electrodepositing a thin layer of copper upon an appropriate form, stripping the resulting layer of electrodeposited copper from said form and thereby producing a copper starting blank, and progressively passing said starting blank through a copper electrodepositing apparatus in the course of which there is built up on said blank an electrodeposit of copper of a desired thickness.

80 5. The method of manufacturing copper plates or the like which comprises electrodepositing a thin layer of copper upon an appropriate form, stripping the resulting layer of electrodeposited copper from said form and thereby producing a copper starting blank, progressively passing said starting blank through an electrodepositing apparatus and electrodepositing copper thereon to a desired thickness, and progressively withdrawing the resulting plate of electrodeposited copper from said apparatus.

85 6. The method of manufacturing copper plates or the like which comprises electrodepositing a thin layer of copper upon an appropriate rotating form, continuously stripping the resulting layer of electrodeposited copper from said form as the form rotates and thereby producing a copper starting blank of any desired length, and progressively passing said starting blank through a copper electrodepositing apparatus in the course of which there is built upon said blank an electrodeposit of copper of a desired thickness.

90 7. The method of manufacturing copper plates or the like which comprises electrodepositing a thin layer of copper upon an appropriate rotating form, continuously stripping the resulting layer of electrodeposited copper from said form as the form rotates and thereby producing a copper starting blank of any desired length, progressively passing said starting blank through an electrodepositing apparatus and electrodepositing copper thereon to a desired thickness, and progressively withdrawing the resulting plate of electrodeposited copper from said apparatus.

110 120 125 130 8. The method of manufacturing copper plates or the like which comprises electrodepositing a thin layer of copper upon an appropriate rotating cylindrical form partially submerged in a copper electrolyte, con-

tinuously stripping the resulting layer of through a copper electrolyte and electrode-  
electrodeposited copper from said form as positing copper thereon to a desired thick-  
and when the rotation of the form carries ness, and progressively withdrawing the re-  
the electrodeposited copper out of the ele- sulting plate of electrodeposited copper from  
trolyte and thereby producing a copper said apparatus.  
starting blank of any desired length,  
progressively passing said starting blank

CHAS. K. TOPPING.